# EUROPEAN PATENT SPECIFICATION

(11) **EP 4 441 256 B1**
(45) Date of publication and mention of the grant of the patent: **17.06.2026**
(21) Application number: 22839607.3
(22) Date of filing: 02.12.2022
(51) Int. Cl.: C21B 13/10, C22B 1/16, C22B 7/02, F27B 9/24, C21B 13/00, C21B 3/04, F27B 9/08, F27B 9/10, F27B 9/12, F27B 9/20, F27D 3/00

(54) **IRON RECOVERY**
RÜCKGEWINNUNG VON EISEN
RÉCUPÉRATION DE FER

(30) Priority: 02.12.2021 ZA 202109859
(43) Date of publication of application: 09.10.2024
(73) Proprietor: Manic Iron Technology Proprietary Limited, 1748 Lanseria (ZA)
(72) Inventor: BEACHY HEAD, John Peter, 1748 Lanseria (ZA); BECERRA NOVOA, Jorge Octavio, 1748 Lanseria (ZA)
(74) Representative: Seifert, Ruth
(86) International application number: PCT/ZA2022/050065
(87) International publication number: WO 2023/102580

(56) References cited:
- CA-A- 1 244 656
- US-A- 4 784 603
- US-A- 4 974 334

## Description

### BACKGROUND OF THE INVENTION

This invention relates to a method for the recovery of ferrous metals from ferrous ores and, in particular, from ferrous ore fines including ferrous waste materials such as tailings from the mining industry.

In the mining industry, a significant amount of ferrous ore fines is generated. These fines/slimes are often discarded as waste into tailings ponds, containing considerable amounts of ferrous ores. In recent years, interest in recovery of valuable minerals from low-grade ores, slimes, and tailings has increased worldwide. These activities are initiated not only to recover minerals but also to address various environmental issues associated with fine particle treatment.

Various methods, for example CA 1 244 656 A and US 4 784 603 A, have been proposed for the direct recovery of ferrous metals from ferrous ore fines. One such method, of the kind described in US Patent No. 8,613,787B2, discloses the use of a rotary kiln in which devolatized coal and iron ore, in the form of pellets or fines, are fed into the rotary kiln and the kiln is then indirectly heated to a temperature in the range of 1000°C to 1100°C. The reaction which takes place in the kiln proceeds as follows:

Fe_{y}O_{y} + C → xFe + yCO (1)

FeₓO_{y} + CO → xFe + yCO₂ (2)

CO₂ + C → 2CO (3)

The CO produced in reaction (3) will continue reacting as indicated in reaction (2).

While the direct reduction of iron ore and iron ore fines is possible using a rotary kiln, this process does have limitations. As the kiln is heated indirectly, there is a constraint in the reduction temperature due to construction materials of the kiln and the size required for an industrial production. Very high temperatures cannot be reached and typically the temperature will be less than 1050°C.

Furthermore, during the devolitilization of coal, the required energy is supplied by direct heating of the coal by partial combustion of the volatile gas. This results in several disadvantages. Firstly, a variable quality of gases is produced which makes its further utilization very complicated. Secondly, there is no way to control the flame inside the devolatilization kiln which results in localized areas of high temperature that damage the equipment as a result of flame impingement.

Once the iron ore has been reduced, the resulting direct reduced iron, ashes and char are cooled. However, the mix of these heterogeneous materials makes indirect cooling a difficult task.

A need therefore exists to provide an alternative method of reducing ferrous ore fines, in an energy efficient manner, which allows higher temperatures to be reached and better control of the process.

The invention aims, at least partially, to achieve these objectives.

### SUMMARY OF INVENTION

The invention provides a method of reducing ferrous metal fines derived from waste or from ferrous ore, the method including the steps of:
a) feeding a fine ferrous material with a particle size distribution of between 10 microns to less than 6mm and a reductant into an indirectly heated vibratory bed furnace; and
b) contacting the fine ferrous material with the reductant in the indirectly heated vibratory bed furnace at a temperature of up to 1350°C to produce a hot direct reduced ferrous metal.

Preferably the fine ferrous material has a size of less than 500 microns. The ferrous ore may be chromite, iron oxide or manganese fines.

Preferably the temperature in step (b) is in the range of 1000°C to 1350°C, more preferably, 1200°C to 1350°C.

The method may include a first preliminary step of preheating the fine ferrous material to a temperature of between 400°C to 500°C to remove excess moisture and to reduce the energy demand in the reduction bed.

The reductant may be a carbon-containing material such as coal. The carbon-containing material may have a particle size distribution of less than 1mm.

If the reductant is coal, the method may include a second preliminary step of devolatilization of the coal through indirect heating with combustion gases to produce char. The char may then be fed into a reduction bed of the furnace. This is done without cooling the char in order to reduce the energy demand of the reduction bed.

The volatile combustible gases produced due to the devolatilization of coal in the second preliminary step and in step (b) may proceed to a gasometer. The combustible gases may be cooled and cleaned prior to passing into the gasometer. The purpose of the gasometer is to provide several steps in the process which use the combustible gases with a more stable gas composition and with a stable flow according to the demand. The gases from the gasometer may be used in the second preliminary step, step (b) and in a subsequent recovery step.

The method may also include the step of recovering sensible heat from combustible gases emitted as a result of devolatilization of the coal to be used to preheat the combustion gases used in the second preliminary step. Sensible heat may also be recovered from combustible gases produced in step (b) to be used to preheat combustion gases for use in the furnace.

The method may include an additional recovery step (c) wherein the hot direct reduced ferrous metal is indirectly heated in a melting unit together with combustion gases produced by burning fuel from the gasometer with preheated air to a temperature of about 2000°C to produce a liquid ferrous metal and a liquid slag.

The liquid ferrous metal may be sent to a granulator to produce a granulated ferrous metal.

The liquid slag may be used as an aggregate substitute or as an extender in a cement manufacturing process. Alternatively, the liquid slag may be sent to waste.

If coal is used as a reductant in step (b), the char and fine ferrous material may be fed into the vibratory bed furnace at a controlled ratio which depends on the quality of material used and the excess of reductant needed to meet the desired carbon content in the liquid ferrous metal.

The residence time of the char and the ferrous fines in the reduction bed of the furnace may be controlled to achieve the desired degree of reduction. The residence time is dependent on the fines characteristics and on the operating temperature. Preferably the residence time is below 15 minutes.

The use of the vibratory bed furnace allows vibrations and combustible gas evolution to create interstitial space to promote solid/solid and solid/gas reduction reactions within the furnace. The vibration action lifts the burden within the furnace to create interstitial space to allow gas movement and to promote the reduction reactions within the furnace.

The vibratory bed furnace may of the kind described below.

The invention further extends to a furnace which comprises a structure in which is formed a production chamber, at least one inlet port for feeding product to be processed into the production chamber, at least one discharge port through which processed product is discharged from the production chamber, a heating arrangement configured to heat product which is in the production chamber to a predetermined temperature and a mechanism which is configured and which is operative to impart controlled vibratory movement to the production chamber and to the product in the production chamber.

The product which is to be processed is typically in fine particulate form. A primary function of the vibratory mechanism is to impart vibratory movement to the production chamber and hence to the particulate material in the production chamber so that, in effect; a suspension of the particulate material in the prevailing atmosphere is achieved. In this way, each particle is effectively removed or displaced from surrounding particles and its surface is fully exposed and hence the particle can then present a maximum surface area to enable reduction to take place.

In one form of the invention the product to be processed is ferrous oxide with a particle size of less than 500 microns.

The heating arrangement should be configured to heat the product in the production chamber to an operating temperature of up to 1350°C.

Through the vibratory movement the particles of the production chamber are thereby interstitially spaced from one another.

The heating arrangement is preferably at a location which is below the production chamber. The inlet port may be at or near a first end of the production chamber. The discharge port may be at or near a second end of the production chamber which is remote from the first end.

The structure may include an outlet from the production chamber through which combustible gas, produced upon heating and hence the reduction of the product in the production chamber, is directed.

The combustible gases may be directed to a gasometer and from there to a combustion system and hot combusted gas from the combustion system may be employed in the heating arrangement.

In the present invention, the structure is mounted to a frame with a vibratory mechanism between the frame and the structure. The vibratory mechanism includes rubber vibratory suspension elements between the frame and the structure.

Through the use of a suitable actuator using techniques which are known in the art, vibratory movement is imparted to the structure which causes the structure to move up and down in a generally vertical direction relative to the frame.

In one respect the particles in the production chamber are aerated by forcing interstitial spacing and the particles are thereby effectively placed in what may be regarded as a suspension.

In one form of construction, the production chamber is located in an upper housing and the heating arrangement is located in a lower housing positioned below the upper housing with a refractory medium between the housings.

### DESCRIPTION OF THE DRAWINGS

The invention is further described by way of example with reference to the accompanying drawings in which:
Figure 1 is a view in perspective from above of a furnace according to one form of the invention;
Figure 2 is a side view of the furnace shown in Figure 1;
Figure 3 illustrates a method of recovering ferrous metals from ferrous ore according to the invention; and
Figure 4 illustrates a ferrous metal recovery step according to the method of the invention.

### DESCRIPTION OF PREFERRED EMBODIMENTS

Figure 1 of the accompanying drawing illustrates a furnace 10 according to the invention. Figure 2 shows the furnace 10 from one side and in cross-section.

The furnace 10 comprises a structure 12 which is mounted to a base frame 14.

The structure 12 comprises an upper housing 18 and a lower housing 20. The two housings are separated by a hot face refractory medium 24.

The upper housing 18 encloses a production chamber 30. A downwardly inclined inlet port 32 is formed close to a first end 34 of the production chamber 30. A discharge port 38 is formed close to a second end 40 of the production chamber 30. The second end 40 is remote from the first end 34. An outlet 44 is formed in an upper wall 46 of the upper housing. Insulating refractory material 50 surrounds the production chamber 30 as may be appropriate.

The hot face refractory medium 24 extends downwardly from the upper housing 18 into the lower housing 20. The lower housing embodies a heating arrangement for product in the upper housing. Heating is achieved by means of a hot combusted gas which is introduced through an inlet 54 and which exits the lower housing through a gas discharge port 56 which is displaced from the inlet 54.

The structure 12 is mounted to an upper support frame 60 upon which the structure rests. Vibratory suspension elements 62 made from rubber or equivalent material are positioned between the upper support frame 60 and a lower support frame 66 which rests on the ground. Through the use of an actuator (not shown) using techniques which are known in the art, up-down vibratory movement, in a generally vertical sense, can be imparted to the structure so that it is moved in an up-down generally vertical sense relative to the lower support frame 66 as is indicated by double-headed arrows 70.

An examination of Figure 2 shows that a base 72 of the production chamber 30 is inclined downwardly moving away from the inlet port 32 to the discharge port 38.

In use of the furnace, ferrous oxide fines 80 with a particle size of less than 500 microns are fed at a controlled rate from a source through the inlet port 32 into the production chamber 30. Hot combusted gas 84 produced by a gas combustion process 86 is fed at a controlled rate into the heating arrangement embodied in the lower housing 20 through the inlet port 54. An objective in this respective is to use the hot combusted gas 84 to heat the product in the production chamber 30 to a temperature of up to 1350°C. Gas which leaves the lower housing is discharged through the port 56.

Ferrous ore particles and char comprise the product feed. The indirect heating process carried out in the lower housing 20 by the hot combusted gas 84 causes the ferrous ore and the char to react and the ferrous is directly reduced to produce high metallization metal fines.

In the reduction process the ferrous oxides are reduced via CO producing CO₂. The CO₂ reacts with the carbon in the char as to produce 2CO and the CO is again used for reduction.

Gases which are produced as a result of the reduction process are very rich in CO which is combustible and are exhausted through the outlet 44 and then directed to the combustion process 86 through the gasometer and fuel gas handling system.

Figure 3 illustrates a method 100 of recovering ferrous metals, from ferrous fines according to the invention.

In a first preliminary step, ferrous fines 102 are heated (104) to a temperature of 400°C to 500°C in order to remove excess moisture to provide a dry ore product 106. The ferrous fines have a size in the range of 10 microns to 6mm. Preferably, the ferrous fines have a size of less than 500 microns.

Coal 108 is also heated (110) in order to remove excess moisture to provide a dry coal product 112. If the coal is coarse, the coal is ground to a size of less than 1mm prior to heating.

In a second preliminary step, the dry coal 112 is subject to a devolatilization step 114 wherein the coal 112 is heated indirectly to remove volatile matter to provide a hot char product 116 and volatile gas 118.

The hot dry fines product 106 and the hot char product 116 are fed into a reduction unit in the form of a vibratory bed furnace 120 in a ratio to be controlled according to the specific properties and quality of the fines and the char as well as to the desired carbon content in the final granulated ferrous product. Preferably, the vibratory bed furnace is of the kind described herein. The furnace 120 is indirectly heated to a temperature of up to 1350°C for a process retention time of preferably less than 15 minutes to produce a hot direct reduced ferrous product 122 and combustible gas 124.

The gasses 118 and 124 are cooled and cleaned and are send to a gasometer 126. The gas from the gasometer 126 is combusted with preheated air 128 in a combustion chamber 130 to provide hot combusted gases which are used to indirectly heat the coal 112 in the devolatilization step 114.

The gasses from the gasometer are also combusted with preheated air 132 in a combustion chamber 134 to provide hot combustion gases which are used to indirectly heat the burden in the vibratory bed furnace 120.

The remaining sensible heat from the combustion gas used in the furnace 120 is used in the heat exchanger 132 to preheat the combustion air for use in the combustion chamber 134. The remaining sensible heat in the combustion gas used in the devolatilization unit 114 is used to preheat the combustion air to be used in the combustion chamber 130 in the heat exchanger 128.

Figure 4 illustrates a ferrous recovery step 140 according to the invention. The hot direct reduced ferrous 122 product is indirectly heated in a melting unit 142 together with gases stored in the gasometer 126 and combusted in the combustion chamber 150 to a temperature of about 2000°C. By indirect contact with the combustion gases, a liquid ferrous product 146 and a liquid slag 144 are produced. The remaining sensible heat from the combustion gases used in the melting unit 142 is used to preheat the combustion air used in the combustion chamber 150 through a heat exchanger 148.

The liquid ferrous metal is sent to a granulator to produce a granulated ferrous product. The liquid slag is used as an aggregate substitute or an extender in a cement manufacturing process, or is sent to waste.

## Claims

1. A method of reducing ferrous metal fines derived from waste or from ferrous ore, the method including the steps of:
a) feeding a fine ferrous material with a particle size distribution of between 10 microns to less than 6mm and a reductant into an indirectly heated vibratory bed furnace;
b) contacting the fine ferrous material with the reductant in the indirectly heated vibratory bed furnace at a temperature of up to 1350°C to produce a hot direct reduced ferrous metal;
and wherein the vibratory bed furnace creates a vibratory action which lifts the burden within the furnace to create interstitial spaces to allow gas movement and to promote the reduction reactions within the furnace.

2. A method according to claim 1 wherein the fine ferrous material has a size of less than 500 microns.

3. A method according to claim 1 or 2 wherein the ferrous ore is selected from one or more of chromite, iron oxide or manganese fines.

4. A method according to any one of claims 1 to 3 wherein the temperature in step (b) is in the range of 1000°C to 1350°C.

5. A method according to any one of claims 1 to 4 which includes a first preliminary step of preheating the fine ferrous material to a temperature of between 400°C to 500°C.

6. A method according to any one of claims 1 to 5 wherein the reductant is a carbon-containing material having a particle size distribution of less than 1mm.

7. A method according to claim 6 wherein the carbon-containing material is coal.

8. A method according to claim 7 which includes a second preliminary step of devolatilization of the coal through indirect heating with combustion gases to produce char.

9. A method according to claim 8 wherein volatile combustible gases produced in the second preliminary step and in step (b) proceed to a gasometer.

10. A method according to claim 9 wherein the gases from the gasometer are used in the second preliminary step, step (b) and in a subsequent recovery step.

11. A method according to claim 10 which includes the step of recovering sensible heat from combustible gases emitted as a result of devolatilization of the coal to be used to preheat the combustion gases used in the second preliminary step.

12. A method according to any one of claims 8 to 11 which includes an additional recovery step (c) wherein the hot direct reduced ferrous metal is indirectly heated in a melting unit together with combustion gases produced by burning fuel from the gasometer with preheated air to a temperature of about 2000°C to produce a liquid ferrous metal and a liquid slag.

13. A method according to claim 8 wherein the residence time of the char and the ferrous fines in the vibratory bed furnace is below 15 minutes.

14. A furnace for use in the method of claim 1 which comprises a structure in which is formed a production chamber, at least one inlet port for feeding product to be processed into the production chamber, at least one discharge port through which processed product is discharged from the production chamber, a heating arrangement configured to heat product which is in the production chamber to a predetermined temperature, wherein the structure is mounted to a frame with a vibratory mechanism between the frame and the structure which is configured and which is operative to impart controlled vibratory movement to the production chamber and to the product in the production chamber and wherein the vibratory mechanism includes rubber vibratory suspension elements between the frame and the structure.

15. A furnace according to claim 14 or 15 wherein the heating arrangement is at a location which is below the production chamber.

16. A furnace according to claim 14 or 15 wherein the inlet port is at a first end of the production chamber and the discharge port is at a second end of the production chamber which is remote from the first end.

17. A furnace according to any one of claims 14 to 16 wherein the structure includes an outlet from the production chamber through which combustible gas, produced upon heating and hence the reduction of the product in the production chamber, is directed.

18. A furnace according to any one of claims 14 to 17 wherein through the vibratory movement the particles in the production chamber are interstitially spaced from one another.

19. A furnace according to any one of claims 14 to 18 the production chamber is located in an upper housing and the heating arrangement is located in a lower housing positioned below the upper housing with a refractory medium between the housings.

## Patentansprüche

1. Verfahren zum Reduzieren von Eisenmetallfeinstoffen, die aus Abfall oder aus Eisenerz stammen, wobei das Verfahren die folgenden Schritte umfasst:
a) Zuführen eines feinen Eisenmaterials mit einer Partikelgrößenverteilung zwischen 10 Mikrometern und weniger als 6 mm und eines Reduktionsmittels in einen indirekt beheizten Vibrationsbettofen;
b) Kontaktieren des feinen Eisenmaterials mit dem Reduktionsmittel in dem indirekt beheizten Vibrationsbettofen bei einer Temperatur von bis zu 1350 °C, um ein heißes, direkt reduziertes Eisenmetall herzustellen;
und wobei der Vibrationsbettofen eine Vibrationswirkung erzeugt, die die Last innerhalb des Ofens anhebt, um interstitielle Räume zu erzeugen, die eine Gasbewegung ermöglichen und die Reduktionsreaktionen innerhalb des Ofens fördern.

2. Verfahren gemäß Anspruch 1, wobei das feine Eisenmaterial eine Größe von weniger als 500 Mikrometern hat.

3. Verfahren gemäß Anspruch 1 oder 2, wobei das Eisenerz aus einem oder mehreren aus Chromit, Eisenoxid oder Manganfeinstoff ausgewählt ist.

4. Verfahren gemäß einem der Ansprüche 1 bis 3, wobei die Temperatur in Schritt (b) in dem Bereich von 1000 °C bis 1350 °C ist.

5. Verfahren gemäß einem der Ansprüche 1 bis 4, das einen ersten vorläufigen Schritt des Vorheizens des feinen Eisenmaterials auf eine Temperatur zwischen 400 °C bis 500 °C umfasst.

6. Verfahren gemäß einem der Ansprüche 1 bis 5, wobei das Reduktionsmittel ein kohlenstoffhaltiges Material mit einer Partikelgrößenverteilung von weniger als 1 mm ist.

7. Verfahren gemäß Anspruch 6, wobei das kohlenstoffhaltige Material Kohle ist.

8. Verfahren gemäß Anspruch 7, das einen zweiten vorläufigen Schritt der Entgasung der Kohle durch indirektes Erhitzen mit Verbrennungsgasen umfasst, um Holzkohle herzustellen.

9. Verfahren gemäß Anspruch 8, wobei flüchtige brennbare Gase, die im zweiten vorläufigen Schritt und in Schritt (b) hergestellt werden, zu einem Gasometer weitergeleitet werden.

10. Verfahren gemäß Anspruch 9, wobei die Gase aus dem Gasometer im zweiten vorläufigen Schritt, in Schritt (b) und in einem nachfolgenden Rückgewinnungsschritt verwendet werden.

11. Verfahren gemäß Anspruch 10, das den Schritt der Rückgewinnung von fühlbarer Wärme aus brennbaren Gasen umfasst, die als Folge der Entgasung der Kohle freigesetzt werden, die verwendet werden, um die im zweiten vorläufigen Schritt verwendeten Verbrennungsgase vorzuwärmen.

12. Verfahren gemäß einem der Ansprüche 8 bis 11, das einen zusätzlichen Rückgewinnungsschritt (c) umfasst, wobei das heiße direkt reduzierte Eisenmetall in einer Schmelzeinheit zusammen mit Verbrennungsgasen, die durch Verbrennen von Brennstoff aus dem Gasometer mit vorgewärmter Luft hergestellt werden, auf eine Temperatur von etwa 2000 °C indirekt erhitzt wird, um ein flüssiges Eisenmetall und eine flüssige Schlacke herzustellen.

13. Verfahren gemäß Anspruch 8, wobei die Verweildauer der Holzkohle und des Eisenfeinstoffs im Vibrationsbettofen unter 15 Minuten ist.

14. Ofen zur Verwendung in dem Verfahren von Anspruch 1, der eine Struktur umfasst, in der eine Produktionskammer, zumindest eine Einlassöffnung zum Zuführen des zu verarbeitenden Produkts in die Produktionskammer, zumindest eine Auslassöffnung, durch die das verarbeitete Produkt aus der Produktionskammer abgegeben wird, eine Heizvorrichtung gebildet ist, die ausgebildet ist, um das in der Produktionskammer befindliche Produkt auf eine vorbestimmte Temperatur zu erhitzen, wobei die Struktur an einem Rahmen mit einem Vibrationsmechanismus zwischen dem Rahmen und der Struktur befestigt ist, der ausgebildet ist und betriebsfähig ist, um der Produktionskammer und dem Produkt in der Produktionskammer eine kontrollierte Vibrationsbewegung zu erteilen, und wobei der Vibrationsmechanismus Gummivibrationsaufhängungselemente zwischen dem Rahmen und der Struktur umfasst.

15. Ofen gemäß Anspruch 14 oder 15, wobei die Heizvorrichtung an einer Stelle ist, die unter der Produktionskammer ist.

16. Ofen gemäß Anspruch 14 oder 15, wobei die Einlassöffnung an einem ersten Ende der Produktionskammer ist und die Auslassöffnung an einem zweiten Ende der Produktionskammer ist, das vom ersten Ende entfernt ist.

17. Ofen gemäß einem der Ansprüche 14 bis 16, wobei die Struktur einen Auslass aus der Produktionskammer umfasst, durch den brennbares Gas, das beim Erhitzen und damit bei der Reduktion des Produkts in der Produktionskammer entsteht, geleitet wird.

18. Ofen gemäß einem der Ansprüche 14 bis 17, wobei durch die Vibrationsbewegung die Partikel in der Produktionskammer in interstitiell voneinander beabstandet sind.

19. Ofen gemäß einem der Ansprüche 14 bis 18, wobei sich die Produktionskammer in einem oberen Gehäuse befindet und sich die Heizvorrichtung in einem unteren Gehäuse befindet, das unterhalb des oberen Gehäuses angeordnet ist, wobei sich zwischen den Gehäusen ein hitzebeständiges Medium befindet.

## Revendications

1. Procédé de réduction de fines métalliques ferreuses tirées de déchets ou du minerai de fer, le procédé comprenant les étapes consistant à :
a) alimenter un matériau ferreux fin avec une distribution de taille de particules comprises entre 10 microns et moins de 6 mm et un agent réducteur dans un four à lit vibratoire chauffé de manière indirecte ;
b) la mise en contact du matériau ferreux fin avec l'agent réducteur dans le four à lit vibratoire indirectement chauffé à une température pouvant atteindre 1350 °C afin de produire un métal ferreux réduit direct chaud ;
et dans lequel le four à lit vibratoire crée une action vibratoire qui lève la charge dans le four afin de créer des espaces interstitiels pour permettre le mouvement du gaz et promouvoir les réactions de réduction dans le four.

2. Procédé selon la revendication 1, dans lequel le matériau ferreux fin présente une taille inférieure à 500 microns.

3. Procédé selon la revendication 1 ou 2 dans lequel le minerai de fer est sélectionné à partir d'un ou plusieurs parmi les fines de chromite, d'oxyde de fer ou de manganèse.

4. Procédé selon l'une quelconque des revendications 1 à 3, dans lequel la température dans l'étape (b) est dans la plage de 1000 °C à 1350 °C.

5. Procédé selon l'une quelconque des revendications 1 à 4, qui comprend une première étape préliminaire consistant à préchauffer le matériau ferreux fin à une température comprise entre 400°C et 500°C.

6. Procédé selon l'une quelconque des revendications 1 à 5, dans lequel l'agent réducteur est un matériau contenant du carbone présentant une distribution de taille de particules inférieure à 1 mm.

7. Procédé selon la revendication 6, dans lequel le matériau contenant du carbone est de la houille.

8. Procédé selon la revendication 7, qui comprend une deuxième étape préliminaire de dévolatilisation de la houille par un chauffage indirect avec des gaz de combustion pour produire du charbon.

9. Procédé selon la revendication 8, dans lequel des gaz combustibles volatils produits dans la deuxième étape préliminaire et dans l'étape (b) s'écoulent vers un gazomètre.

10. Procédé selon la revendication 9, dans lequel les gaz provenant du gazomètre sont utilisés dans la deuxième étape préliminaire, l'étape (b) et dans une étape de récupération successive.

11. Procédé selon la revendication 10 qui comprend l'étape consistant à récupérer la chaleur sensible des gaz combustibles émis du fait d'une dévolatilisation de la houille utilisée pour préchauffer les gaz de combustion utilisés dans la deuxième étape préliminaire.

12. Procédé selon l'une quelconque des revendications 8 à 11, qui comprend une étape de récupération supplémentaire (c) dans lequel le métal ferreux réduit direct chaud est indirectement chauffé dans une unité de mélange avec des gaz de combustion produits par la combustion du combustible provenant du gazomètre avec de l'air préchauffé à une température d'environ 2000 °C afin de produire un métal ferreux liquide et une scorie liquide.

13. Procédé selon la revendication 8, dans lequel le temps de séjour du charbon et des fines ferreuses dans le four à lit vibratoire est inférieur à 15 minutes.

14. Four pour une utilisation dans le procédé selon la revendication 1, qui comprend une structure dans laquelle une chambre de production est formée, au moins un orifice d'entrée pour alimenter un produit à traiter dans la chambre de production, au moins un orifice de décharge à travers lequel le produit traité est déchargé de la chambre de production, un agencement de chauffage configuré pour chauffer le produit qui se trouve dans la chambre de production à une température prédéterminée, dans lequel la structure est montée sur un châssis avec un mécanisme vibratoire entre le châssis et la structure qui est configurée et qui est opérationnelle pour donner un mouvement vibratoire contrôlé à la chambre de production et au produit dans la chambre de production et dans lequel le mécanisme vibratoire comprend des éléments de suspension vibratoires en caoutchouc entre le châssis et la structure.

15. Four selon la revendication 14 ou 15, dans lequel l'agencement de chauffage se situe à un endroit sous la chambre de production.

16. Four selon la revendication 14 ou 15, dans lequel l'orifice d'entrée est à une première extrémité de la chambre de production et l'orifice de décharge est à une seconde extrémité de la chambre de production qui est distante de la première extrémité.

17. Four selon l'une quelconque des revendications 14 à 16, dans lequel la structure comprend une sortie de la chambre de production à travers laquelle le gaz combustible, produit lors du chauffage et donc de la réduction du produit dans la chambre de production, est dirigé.

18. Four selon l'une quelconque des revendications 14 à 17, dans lequel le mouvement vibratoire des particules dans la chambre de production sont espacées de manière interstitielle les unes des autres.

19. Four selon l'une quelconque des revendications 14 à 18 dans lequel la chambre de production est située dans un logement supérieur et l'agencement de chauffage est situé dans un logement inférieur positionné sous le logement supérieur avec un milieu réfractaire entre les logements.
